

2,826,498

## TITANIUM-SULFUR BASE ALLOYS

Harry P. Croft, Green Farms, Conn., assignor to Kennecott Copper Corporation, New York, N. Y., a corporation of New York

No Drawing. Application October 21, 1955  
Serial No. 542,105

6 Claims. (Cl. 75—175.5)

This invention relates to titanium alloys and more particularly to titanium-sulfur alloys and titanium-sulfur base alloys. It further relates to a method for providing titanium-sulfur base alloys wherein alloying additions are introduced into the titanium in the form of appropriate sulfides.

In the past it has been shown that the addition of small amounts of sulfur to titanium produces alloys having improved strength and ductility properties as compared with unalloyed titanium metal. Such alloys are described in my copending application Serial No. 297,125, filed July 3, 1952, now Patent No. 2,721,797, granted October 25, 1955, of which this application is a continuation-in-part. It has now been found that useful alloys of titanium and sulfur may be produced through the addition of sulfur in considerably higher amounts than were contemplated in the prior art. Still further, it has been found that extremely valuable ternary and quaternary titanium-sulfur base alloys can be produced and particularly that such alloys can conveniently be prepared by adding appropriate sulfides to titanium metal in an alloying process.

It is, therefore, an object of this invention to provide useful binary alloys of titanium and sulfur containing increased amounts of sulfur as compared with prior art alloys.

Another object of this invention is to provide valuable titanium-sulfur base alloys.

Still another object of this invention is to provide a method for preparing titanium-sulfur base alloys, wherein alloying additions are made in the form of sulfides.

Yet another object of this invention is to provide titanium-sulfur base alloys having good properties of strength, hot hardness, and heat treatability.

Other objects and advantages of the invention will be apparent from the following detailed description thereof.

In general, this invention comprises titanium-sulfur alloys and titanium-sulfur base alloys and a method for preparing such alloys.

It has been found that high-strength, heat-treatable alloys can be prepared by adding sulfur as a metal sulfide to titanium metal. Similarly valuable binary alloys of titanium and sulfur can be prepared by adding titanium sulfide to titanium metal in quantity sufficient to provide binary alloys containing from 1 to 20 percent sulfur.

Table 1 below shows the effect of sulfur additions on the as-cast hardness of commercial purity titanium. It will be apparent from the values listed that titanium-sulfur binary alloys possess high hardness rendering them useful for the many applications where such hardness is important—for example in the tool industry.

TABLE 1

| Composition, <sup>1</sup> weight percent |  | As-cast<br>Vickers<br>hardness<br>(10 kg.<br>load) |
|------------------------------------------|--|----------------------------------------------------|
| 100 Ti                                   |  | 161                                                |
| Ti—0.96S                                 |  | 266                                                |
| Ti—1.90S                                 |  | 357                                                |
| Ti—2.86S                                 |  | 387                                                |
| Ti—5.0S                                  |  | 429                                                |
| Ti—10.0S                                 |  | 649                                                |
| Ti—15.0S                                 |  | 762                                                |
| Ti—20.0S                                 |  | 933                                                |

<sup>1</sup> Sulfur added as titanium sulfide.

TABLE 2

| Sulfide<br>addition,<br>weight<br>percent | Composition, weight<br>percent | Tensile<br>strength,<br>p. s. i. | Yield strength,<br>p. s. i. |                | Elongation,<br>percent in<br>1 inch |       | Re-<br>duc-<br>tion<br>in<br>area,<br>per-<br>cent | Vickers<br>hardness<br>(10 kg.<br>load) | Bend<br>ductility,<br>T |
|-------------------------------------------|--------------------------------|----------------------------------|-----------------------------|----------------|-------------------------------------|-------|----------------------------------------------------|-----------------------------------------|-------------------------|
|                                           |                                |                                  | 0.1%<br>offset              | 0.2%<br>offset | Uni-<br>form                        | Total |                                                    |                                         |                         |
|                                           |                                |                                  |                             |                |                                     |       |                                                    |                                         |                         |
| None                                      | 100 Ti Cu                      | 67,000                           | 45,000                      | 48,000         | 15                                  | 31    | 53                                                 | 176                                     | 0                       |
| 1Cu <sub>2</sub> S                        | Ti—0.8—0.2S                    | 82,000                           | 63,000                      | 64,000         | 14                                  | 27    | 38                                                 | 206                                     | 1.7                     |
| 2Cu <sub>2</sub> S                        | Ti—1.6Cu—0.4S                  | 86,000                           | 65,000                      | 67,000         | 12                                  | 21    | 29                                                 | 224                                     | 2.5                     |
| 4Cu <sub>2</sub> S                        | Ti—3.2Cu—0.8S                  | 103,000                          | 77,000                      | 79,000         | 12                                  | 17    | 21                                                 | 247                                     | 4.0                     |
| 6Cu <sub>2</sub> S                        | Ti—4.8Cu—1.2S                  | 114,000                          | 84,000                      | 88,000         | 11                                  | 13    | 17                                                 | 272                                     | 5.0                     |
| 1Cr <sub>2</sub> S <sub>3</sub>           | Ti—0.53Cr—0.47S                | 83,000                           | 62,000                      | 63,000         | 14                                  | 23    | 35                                                 | 216                                     | 1.8                     |
| 2Cr <sub>2</sub> S <sub>3</sub>           | Ti—1.05Cr—0.96S                | 93,000                           | 76,000                      | 76,000         | 12                                  | 20    | 31                                                 | 219                                     | 2.8                     |
| 4Cr <sub>2</sub> S <sub>3</sub>           | Ti—2.1Cr—1.9S                  | 103,000                          | 90,000                      | 92,000         | 7                                   | 7     | 7                                                  | 253                                     | 19.3                    |
| 1FeS                                      | Ti—0.63Fe—0.36S                | 84,000                           | 59,000                      | 60,000         | 15                                  | 27    | 34                                                 | 202                                     | 1.5                     |
| 2FeS                                      | Ti—1.27Fe—0.73S                | 99,000                           | 70,000                      | 72,000         | 14                                  | 22    | 31                                                 | 232                                     | 1.8                     |
| 4FeS                                      | Ti—2.55Fe—1.48S                | 116,000                          | 92,000                      | 93,000         | 9                                   | 9     | 12                                                 | 279                                     | 5.2                     |
| 1MoS <sub>2</sub>                         | Ti—0.6Mo—0.4S                  | 85,000                           | 69,000                      | 70,000         | 15                                  | 28    | 44                                                 | 219                                     | 2.2                     |
| 2MoS <sub>2</sub>                         | Ti—1.2Mo—0.8S                  | 94,000                           | 81,000                      | 84,000         | 11                                  | 20    | 37                                                 | 240                                     | 4.6                     |
| 1PbS                                      | Ti—0.86Pb—0.14S                | 78,000                           | 59,000                      | 59,000         | 13                                  | 28    | 37                                                 | 202                                     | 1.9                     |
| 2PbS                                      | Ti—1.73Pb—0.27S                | 89,000                           | 68,000                      | 70,000         | 12                                  | 26    | 37                                                 | 233                                     | 1.8                     |
| 4PbS                                      | Ti—3.46Pb—0.54S                | 100,000                          | 82,000                      | 83,000         | 11                                  | 21    | 33                                                 | 281                                     | 2.6                     |
| 6PbS                                      | Ti—5.19Pb—0.81S                | 110,000                          | 91,000                      | 93,000         | 11                                  | 18    | 25                                                 | 302                                     | 2.6                     |
| 1SnS                                      | Ti—0.79Sn—0.21S                | 74,000                           | 55,000                      | 55,000         | 16                                  | 29    | 40                                                 | 191                                     | 1.8                     |
| 2SnS                                      | Ti—1.58Sn—0.42S                | 77,000                           | 58,000                      | 59,000         | 12                                  | 23    | 31                                                 | 202                                     | 1.9                     |
| 4SnS                                      | Ti—3.16Sn—0.84S                | 82,000                           | 65,000                      | 66,000         | 11                                  | 20    | 30                                                 | 221                                     | 1.9                     |
| 1MnS                                      | Ti—0.63Mn—0.37S                | 79,000                           | 59,000                      | 60,000         | 15                                  | 24    | 38                                                 | 193                                     | 1.3                     |
| 2MnS                                      | Ti—1.25Mn—0.75S                | 92,000                           | 68,000                      | 69,000         | 14                                  | 24    | 29                                                 | 215                                     | 2.2                     |
| 4MnS                                      | Ti—2.5Mn—1.5S                  | 110,000                          | 91,000                      | 91,000         | 5                                   | 5     | 8                                                  | 253                                     | 4.9                     |
| 1WS <sub>2</sub>                          | Ti—0.76W—0.24S                 | 88,000                           | 66,000                      | 68,000         | 15                                  | 32    | 43                                                 | 193                                     | 0.8                     |
| 2WS <sub>2</sub>                          | Ti—1.52W—0.48S                 | 99,000                           | 79,000                      | 82,000         | 14                                  | 22    | 39                                                 | 219                                     | 2.8                     |
| 0.5Al <sub>2</sub> S <sub>3</sub>         | Ti—0.20Al—0.30S                | 85,000                           | 64,000                      | 66,000         | 14                                  | 30    | 39                                                 | 197                                     | 1.7                     |
| 1Al <sub>2</sub> S <sub>3</sub>           | Ti—0.39Al—0.61S                | 99,000                           | 78,000                      | 80,000         | 14                                  | 28    | 37                                                 | 236                                     | 1.7                     |
| 2Al <sub>2</sub> S <sub>3</sub>           | Ti—0.78Al—1.22S                | 131,000                          | 113,000                     | 115,000        | 13                                  | 16    | 17                                                 | 302                                     | 5.7                     |
| 1Ta <sub>2</sub> S <sub>3</sub>           | Ti—0.74Ta—0.26S                | 78,000                           | 57,000                      | 62,000         | 3                                   | —     | 40                                                 | 212                                     | 2.3                     |
| 2Ta <sub>2</sub> S <sub>3</sub>           | Ti—1.48Ta—0.52S                | 89,000                           | 61,000                      | 66,000         | 6                                   | 10    | 33                                                 | 232                                     | 3.1                     |
| 3Ta <sub>2</sub> S <sub>3</sub>           | Ti—2.52Ta—0.78S                | 98,000                           | 73,000                      | 78,000         | 6                                   | 9     | 31                                                 | 238                                     | 2.4                     |
| 4Ta <sub>2</sub> S <sub>3</sub>           | Ti—2.98Ta—1.04S                | 102,000                          | 75,000                      | 80,000         | 6                                   | 7     | 20                                                 | 262                                     | 6.1                     |

Titanium-sulfur base alloys prepared by the addition of metal sulfides to titanium are characterized by good strength and ductility, and by increased hardness as compared with unalloyed titanium. Table 2 above shows the mechanical properties of titanium-sulfur base alloys prepared by sulfide additions to titanium metal. The data in this table were obtained in tests performed on specimens after equilibration and stabilization as follows: Specimens held at 700° C. for 1/2 hour, furnace cooled to 600° C., held at 600° C. for one hour, and air cooled. Specimens tests were approximately 0.040 inch thick. The reduced section of tensile specimens measured 0.25 inch by 1.25 inches.

Titanium-sulfur base alloys prepared as mentioned above have also been found to possess improved hot hardness values as compared with unalloyed titanium metal. Table 3 above lists hot hardness values for such alloys and for temperatures of 300° C., 400° C., 500° C., and 600° C. Values listed in Table 3 were obtained during tests conducted under a vacuum of less than 5 microns using a load of 730 grams and an indentation time of 10 seconds.

Table 4 below shows bend ductility and hardness values for titanium-sulfur base alloys after quenching from tem-

TABLE 4

| Sulfide addition, weight percent | Composition, weight percent | Bend ductility, T, and Vickers hardness, VHN, after quenching from— |     |        |      |        |      |        |      |        |      |
|----------------------------------|-----------------------------|---------------------------------------------------------------------|-----|--------|------|--------|------|--------|------|--------|------|
|                                  |                             | 700 C.                                                              |     | 760 C. |      | 810 C. |      | 870 C. |      | 930 C. |      |
|                                  |                             | VHN                                                                 | T   | VHN    | T    | VHN    | T    | VHN    | T    | VHN    | T    |
| None                             | 100 Ti                      | 181                                                                 | 0   | 184    | 0    | 182    | 0    | 189    | 0    | 214    | 0    |
| 1Cu <sub>2</sub> S               | Ti-0.48S                    | 226                                                                 | 1.7 | 244    | 2.5  | 234    | 1.7  | 252    | 2.5  | 331    | 9.8  |
| 1Cu <sub>2</sub> S               | Ti-0.8Cu-0.2S               | 216                                                                 | 2.3 | 218    | 3.1  | 226    | 4.8  | 268    | 1.6  | 297    | 2.5  |
| 2Cu <sub>2</sub> S               | Ti-1.6Cu-0.4S               | 236                                                                 | 4.6 | 237    | 4.5  | 238    | 2.3  | 273    | 6.1  | 312    | 4.6  |
| 4Cu <sub>2</sub> S               | Ti-3.2Cu-0.8S               | 259                                                                 | 6.4 | 286    | 5.8  | 325    | 6.1  | 290    | 17.8 | 303    | 19.7 |
| 6Cu <sub>2</sub> S               | Ti-4.8Cu-1.2S               | 284                                                                 | 8.9 | 287    | 17.4 | 334    | 17.8 | 349    | 17.8 | 437    | 17.4 |
| 1Cr <sub>2</sub> S <sub>3</sub>  | Ti-0.53Cr-0.47S             | 199                                                                 | 1.8 | 215    | 1.7  | 225    | 1.8  | 249    | 1.7  | 251    | 1.5  |
| 2Cr <sub>2</sub> S <sub>3</sub>  | Ti-1.05Cr-0.95S             | 234                                                                 | 2.3 | 243    | 4.6  | 261    | 4.7  | 299    | 17.8 | 334    | 18.3 |
| 1FeS                             | Ti-0.63Fe-0.36S             | 224                                                                 | 1.7 | 230    | 1.6  | 237    | 4.9  | 246    | 2.5  | 243    | 4.9  |
| 2FeS                             | Ti-1.27Fe-0.73S             | 230                                                                 | 4.9 | 258    | 2.5  | 299    | 4.7  | 318    | 4.4  | 445    | 18.3 |
| 1MoS <sub>2</sub>                | Ti-0.6Mo-0.4S               | 213                                                                 | 1.5 | 216    | 1.1  | 225    | 1.5  | 252    | 2.2  | 263    | 1.5  |
| 2MoS <sub>2</sub>                | Ti-1.2Mo-0.8S               | 242                                                                 | 2.2 | 252    | 2.1  | 276    | 2.2  | 269    | 13.2 | 326    | 19.2 |
| 1MnS                             | Ti-0.63Mn-0.37S             | 196                                                                 | 0.8 | 197    | 1.7  | 209    | 0.8  | 221    | 1.4  | 224    | 1.7  |
| 2MnS                             | Ti-1.25Mn-0.76S             | 218                                                                 | 1.8 | 242    | 1.7  | 258    | 2.5  | 251    | 2.7  | 266    | 1.7  |
| 4MnS                             | Ti-2.5Mn-1.8S               | 266                                                                 | 5.1 | 294    | 9.6  | 348    | 5.1  | 413    | 18.3 | 357    | 19.6 |

TABLE 3

| Sulfide addition, weight percent  | Composition, weight percent | Vickers hardness, kg./mm. <sup>2</sup> at— |         |         |         |
|-----------------------------------|-----------------------------|--------------------------------------------|---------|---------|---------|
|                                   |                             | 300° C.                                    | 400° C. | 500° C. | 600° C. |
| None                              | 100 Ti                      | 101                                        | 82      | 61      | 38      |
| 1Cu <sub>2</sub> S                | Ti-0.8Cu-0.2S               | 143                                        | 117     | 91      | 56      |
| 2Cu <sub>2</sub> S                | Ti-1.6Cu-0.4S               | 157                                        | 146     | 116     | 68      |
| 4Cu <sub>2</sub> S                | Ti-3.2Cu-0.8S               | 164                                        | 139     | 105     | 60      |
| 6Cu <sub>2</sub> S                | Ti-4.8Cu-1.2S               | 160                                        | 152     | 116     | 61      |
| 1Cr <sub>2</sub> S <sub>3</sub>   | Ti-0.53Cr-0.47S             | 120                                        | 98      | 76      | 42      |
| 2Cr <sub>2</sub> S <sub>3</sub>   | Ti-1.05Cr-0.95S             | 133                                        | 117     | 89      | 50      |
| 4Cr <sub>2</sub> S <sub>3</sub>   | Ti-2.1Cr-1.9S               | 168                                        | 137     | 104     | 63      |
| 6Cr <sub>2</sub> S <sub>3</sub>   | Ti-3.15Cr-2.85S             | 188                                        | 149     | 115     | 68      |
| 1FeS                              | Ti-0.63Fe-0.36S             | 107                                        | 81      | 67      | 38      |
| 2FeS                              | Ti-1.27Fe-0.73S             | 139                                        | 118     | 83      | 44      |
| 4FeS                              | Ti-2.55Fe-1.45S             | 169                                        | 139     | 88      | 45      |
| 1MoS <sub>2</sub>                 | Ti-0.6Mo-0.4S               | 140                                        | 108     | 77      | 46      |
| 2MoS <sub>2</sub>                 | Ti-1.2Mo-0.8S               | 149                                        | 124     | 85      | 46      |
| 2PbS                              | Ti-1.73Pb-0.27S             | 116                                        | 90      | 68      | 44      |
| 4PbS                              | Ti-3.46Pb-0.54S             | 117                                        | 92      | 68      | 42      |
| 6PbS                              | Ti-5.19Pb-0.81S             | 144                                        | 113     | 79      | 54      |
| 4SnS                              | Ti-3.16Sn-0.84S             | 126                                        | 91      | 70      | 50      |
| 1MnS                              | Ti-0.63Mn-0.37S             | 120                                        | 101     | 76      | 43      |
| 2MnS                              | Ti-1.25Mn-0.75S             | 170                                        | 137     | 100     | 49      |
| 4MnS                              | Ti-2.5Mn-1.5S               | 177                                        | 160     | 97      | 45      |
| 1WS <sub>2</sub>                  | Ti-0.76W-0.24S              | 103                                        | 85      | 64      | 39      |
| 2WS <sub>2</sub>                  | Ti-1.52W-0.48S              | 148                                        | 114     | 79      | 50      |
| 0.5Al <sub>2</sub> S <sub>3</sub> | Ti-0.20Al-0.30S             | 108                                        | 81      | 64      | 40      |
| 1Al <sub>2</sub> S <sub>3</sub>   | Ti-0.39Al-0.61S             | 125                                        | 106     | 79      | 51      |
| 2Al <sub>2</sub> S <sub>3</sub>   | Ti-0.78Al-1.22S             | -----                                      | 131     | 101     | 64      |

55

peratures of 700° C., 760° C., 810° C., 870° C., and 930° C. Specimens were held at temperature for one hour and then water quenched.

60 Sheet prepared from titanium-sulfur base alloys exhibits outstanding properties. Table 5 lists mechanical properties of several titanium-sulfur base sheet materials and also includes, for comparison, mechanical properties of some corresponding titanium alloys without the sulfide additions. The Ti-Mo-V-S alloys in particular exhibit outstanding properties. For the alloys in Table 5, sulfur was introduced in the form of MoS<sub>2</sub>. The stabilizing treatment consisted of holding the specimen at 700° C. for 1/2 hour, furnace cooling to 600° C., holding for one hour at 600° C., and air cooling. The "quenched and aged" specimen was held at 730° C. for two hours, water quenched, held at 500° C. for 16 hours, and then air cooled. The results of tests at elevated temperatures (480° C.) show the strengthening effect of the sulfide additions.

TABLE 5  
A. SPECIMENS TESTED AT ROOM TEMPERATURE

| Composition, weight percent | Condition of material tested | Tensile strength, p. s. i. | Yield strength, p. s. i. |             | Elongation, percent in 1 inch |       | Reduction in area, percent | Vickers hardness (10 kg. load) | Bend ductility, T |
|-----------------------------|------------------------------|----------------------------|--------------------------|-------------|-------------------------------|-------|----------------------------|--------------------------------|-------------------|
|                             |                              |                            | 0.1% offset              | 0.2% offset | Uniform                       | Total |                            |                                |                   |
| Ti-4Mo                      | Stabilized                   | 85,000                     | 60,000                   | 66,000      | 8                             | 15    | 39                         | 215                            | 1.4               |
| Ti-4Mo-1/2S                 | do                           | 91,000                     | 68,000                   | 73,000      | 6                             | 11    | 27                         | 240                            | 1.4               |
| Ti-8Mo                      | do                           | 98,000                     | 76,000                   | 83,000      | 6                             | 9     | 17                         | 236                            | 2.2               |
| Ti-8Mo-1/2S                 | do                           | 100,000                    | 79,000                   | 85,000      | 4                             | 6     | 22                         | 258                            | 4.2               |
| Ti-5Cr-1.2Mo-0.8S           | do                           | 123,000                    | 113,000                  | 115,000     | 11                            | 16    | 27                         | 264                            | 7.6               |
| Ti-5V-1.2Mo-0.8S            | do                           | 130,000                    | 113,000                  | 119,000     | 8                             | 8     | 10                         | 281                            | 14.3              |
| Ti-5V-1.2Mo-0.8S            | Quenched and aged            | 150,000                    | 115,000                  | 125,000     | 7                             | 11    | 19                         | 325                            | 2.9               |

B. SPECIMENS TESTED AT 480° C.

|             |            |        |  |  |  |    |    |  |  |
|-------------|------------|--------|--|--|--|----|----|--|--|
| Ti-4Mo      | Stabilized | 41,000 |  |  |  | 12 | 46 |  |  |
| Ti-4Mo-1/2S | do         | 54,000 |  |  |  | 8  | 34 |  |  |
| Ti-8Mo      | do         | 52,000 |  |  |  |    | 18 |  |  |
| Ti-8Mo-1/2S | do         | 60,000 |  |  |  |    | 23 |  |  |
| Ti-8Mo-1/2S | do         | 65,000 |  |  |  | 7  | 24 |  |  |

Sulfur in the form of sulfides added to titanium retards grain growth. This grain-refining effect is illustrated by the data in Table 6 which show the effect of 0.1 percent sulfur on the grain size of commercial purity titanium at 750° C. and 900° C. In obtaining these data, the grain diameters were measured by visual comparison with charts at 100 magnifications.

TABLE 6

| Time at Temperature, Hours | Average Grain Diameter, mm. At Temperature, °C. |       |       |       |
|----------------------------|-------------------------------------------------|-------|-------|-------|
|                            | 750                                             |       | 900   |       |
|                            | Ti                                              | Ti-1S | Ti    | Ti-1S |
| 1/4                        | 0.060                                           | 0.030 | 0.060 | 0.035 |
| 1                          | 0.060                                           | 0.030 | 0.140 | 0.043 |
| 4                          | 0.100                                           | 0.035 | 0.300 | 0.250 |
| 16                         | 0.170                                           | 0.035 | 0.300 | 0.250 |
| 64                         | 0.200                                           | 0.140 |       |       |

In view of the above disclosure it will be apparent that new and useful titanium-sulfur alloys and titanium-sulfur base alloys have been discovered, together with a method of preparing such alloys. Binary alloys of titanium with from about 1 percent to about 20 percent sulfur have been shown to possess improved and desirable hardness properties. Titanium-sulfur base alloys prepared by the addition of sulfides to the titanium metal have been shown to possess good strength and hot hardness properties and to be heat treatable. It has been shown that the effect of sulfur added as a metal sulfide is to impart strength, hot hardness, and heat treatability. Titanium-sulfur base alloys containing from about 0.2 percent to about 20 percent sulfur have been found to possess these desirable strength, hot hardness, and heat treatability characteristics. Alloying metals, added as sulfides, and present in the alloy in amounts from about 0.2 percent to about 10 percent, provide alloys having these same desirable characteristics. Indeed alloying metals in amounts up to 30 percent provide useful alloys as illustrated in Table 7 below, showing the effect of MoS<sub>2</sub> additions on the as-cast hardness of high-purity titanium.

TABLE 7

| MoS <sub>2</sub> addition, weight percent | Composition, weight percent | As-cast Vickers hardness, 10 kg. load |
|-------------------------------------------|-----------------------------|---------------------------------------|
| 0                                         | Unalloyed                   | 100                                   |
| 1.7                                       | 1Mo-0.7S                    | 207                                   |
| 8.4                                       | 5Mo-3.4S                    | 405                                   |
| 16.8                                      | 10Mo-6.8S                   | 540                                   |
| 50.3                                      | 30Mo-20.3S                  | 795                                   |

It has been further shown that the addition of sulfur, as a sulfide, retards grain growth. While it is true that such grain refining effect can be obtained with other elements, carbon, for example, because of the lower solubility of sulfur in titanium, this effect can be obtained at lower sulfur contents than with other refining elements.

The method herein disclosed for preparing titanium-sulfur base alloys, i. e., the addition of sulfur as a sulfide, has a number of advantages, aside from the excellence of the product so obtained. For instance, by this method it is possible to alloy the more volatile metals with titanium by adding such metals as sulfides. A good example of such a metal is lead which may be alloyed with titanium by adding it as lead sulfide (PbS) to the titanium metal.

Titanium-sulfur base alloys having useful and valuable properties have been prepared by adding sulfur as a sulfide such as titanium sulfide, copper sulfide, chromium sulfide, iron sulfide, molybdenum sulfide, manganese sulfide, lead sulfide, tin sulfide, tungsten sulfide, aluminum sulfide, and tantalum sulfide. The exact manner in which alloys have been prepared by sulfide addition is illustrated by the following example:

*Example*

Titanium-sulfur and titanium-sulfur base alloys were prepared by melting in an inert tungsten-electrode arc type furnace. After charging a mixture of titanium and metal sulfide on a water-cooled copper hearth, the furnace was evacuated and flushed with argon several times. Arc melting was done with 250 to 350 amperes of current, after evacuating once again to a static argon pressure of from 15 to 20 centimeters of mercury. The resultant ingot was inverted and remelted several times until homogeneous. During melting, the metal sulfide is reduced, the metal alloying with titanium, and the sulfur combining with titanium to form titanium sulfide.

A titanium-sulfur base alloy of any composition may be prepared by charging an additional amount of alloying metal or metals together with the titanium and metal sulfide. In this manner, any number of ternary, quaternary, and more complex titanium-sulfur base alloys may be prepared which will consist of a matrix of titanium alloy and dispersed titanium sulfide particles.

It will be understood, of course, that useful titanium-sulfur base alloys can be prepared by the addition of metal sulfides other than those specifically mentioned in the examples and disclosure above. It is clear from the number of examples and from the data above that a general method of preparing these alloys has been discovered, such method comprising the addition of metal sulfides to titanium metal to produce titanium-sulfur base alloys. For example, the sulfides of vanadium, cadmium, nickel, cobalt, antimony, bismuth, mercury, silver,

zinc, calcium, indium, cerium, and other metals may be added to titanium metal to provide valuable titanium-sulfur base metals.

New and useful alloys and a method for preparing them having been disclosed, it is desired to further define this invention according to the following claims.

What is claimed is:

1. Titanium-sulfur base alloys consisting essentially of sulfur in amounts ranging from about 0.2 percent to about 20 percent, an alloying metal in an amount ranging from about 0.2 percent to about 10 percent, balance titanium, said alloys being characterized by improved strength and increased hot hardness, as compared with unalloyed titanium, and further characterized by being heat treatable.

2. Titanium-sulfur base alloys consisting essentially of sulfur in amounts ranging from about 0.2 percent to about 20 percent, an alloying metal in an amount ranging from about 0.2 percent to about 20 percent, balance titanium, said sulfur and said alloying metal having been introduced into the alloy melt as a sulfide.

3. Alloys according to claim 2 wherein said sulfur and said alloying metal have been introduced into the alloy melt as a metal sulfide from the group consisting of copper sulfide, chromium sulfide, iron sulfide, molybdenum sulfide, manganese sulfide, lead sulfide, tin sulfide, tungsten sulfide, aluminum sulfide, and tantalum sulfide.

4. Complex titanium-sulfur base alloys comprising from about 0.2 percent to about 20 percent sulfur, at least two alloying metals one of which has been added to the alloy melt as a sulfide, balance titanium.

5. Complex titanium-sulfur base alloys consisting essentially of from about 0.2 percent to about 20 percent sulfur, about 5 percent vanadium, about 1 percent to 1.5 percent molybdenum, said molybdenum having been added in the form of molybdenum sulfide, and balance titanium.

6. A complex titanium-sulfur base alloy consisting essentially of about 0.8 percent sulfur, about 1.2 percent molybdenum, about 5 percent vanadium, balance titanium.

#### References Cited in the file of this patent

#### UNITED STATES PATENTS

|           |         |               |
|-----------|---------|---------------|
| 609,467   | Rossi   | Aug. 23, 1898 |
| 992,423   | Hubbard | May 16, 1911  |
| 1,089,773 | Kraus   | Mar. 10, 1914 |
| 2,721,797 | Croft   | Oct. 25, 1955 |

#### OTHER REFERENCES

Goldhoff, R. M. et al.: "The Influence of Insoluble Phases on the Machinability of Titanium," published as A. S. M. 1952.

U. S. DEPARTMENT OF COMMERCE  
PATENT OFFICE  
CERTIFICATE OF CORRECTION

Patent No. 2,826,498

March 11, 1958

Harry P. Croft

It is hereby certified that error appears in the printed specification of the above numbered patent requiring correction and that the said Letters Patent should read as corrected below.

Column 2, Table 2, under the heading "Composition, weight percent" first two lines thereof, for

100 Ti Cu  
Ti-0.8—0.2S

read

100 Ti  
Ti-0.8Cu-0.2S

Signed and sealed this 22nd day of April 1958.

(SEAL)

Attest:

KARL H. AXLINE

Attesting Officer

ROBERT C. WATSON  
Commissioner of Patents